

## 1

3,546,118

### METAL WORKING OPERATIONS AND LUBRICANTS

Marvin M. Johnson and Paul R. Stapp, Bartlesville, Okla., assignors to Phillips Petroleum Company, a corporation of Delaware  
No Drawing. Filed Nov. 25, 1968, Ser. No. 778,746  
Int. Cl. C10m 1/30

U.S. Cl. 252—54

3 Claims

#### ABSTRACT OF THE DISCLOSURE

Cyclic ethers having the formula



where R is hydrogen or an alkyl or cycloalkyl radical or combination thereof such as alkylcycloalkyl having up to and including 17 carbon atoms and where X is a halogen are lubricants used in metal working operations.

This invention relates to a method of metal working.

There are a number of metal working operations, most of which require the use of a lubricant or a coolant. More and more mechanical devices, engines, etc. are being designed, most of which require lubricants both in production and operation.

Accordingly, an object of this invention is to provide a method of metal working comprising lubricating said metal working operations. Other objects, advantages, features of our invention will become apparent to one skilled in the art from the following disclosure and claims.

We have discovered that a cyclic ether having the formula



where R is hydrogen or an alkyl or cycloalkyl radical or combinations thereof such as alkylcycloalkyl having up to and including 17 carbon atoms and wherein X is a halogen can be employed as a lubricant in metal working operations. Specific examples of such cyclic ethers are 4-chlorotetrahydropyran, 3 - methyl - 4-chlorotetrahydropyran, 3-propyl - 4 - bromotetrahydropyran, 3-amyl-4-chlorotetrahydropyran, 3 - heptyl - 4 - iodotetrahydropyran, 3 - nonyl - 4 - chlorotetrahydropyran, 3-cyclohexyl - 4 - fluorotetrahydropyran, 3-(4-butylcyclohexyl) - 4 - chlorotetrahydropyran, 3 - heptadecyl-4-bromotetrahydropyran, 3 - (2 - propyltetradecyl) - 4-chlorotetrahydropyran, 3 - (4 - cyclohexyldecyl-4-iodotetrahydropyran, 3-(6 - cyclopentyldecyl) - fluorotetrahydropyran, and the like. The lubricants of this invention provide reduced galling and dragging tendencies in these metal working operations.

## 2

Typical metal working operations are cutting, machining, grinding, molding, forging, rolling, threading, and the like. Lubricants of this invention are particularly useful in metal working operations such as cutting, cutting threads, threading, and the like.

5 The cyclic ether lubricants of this invention can be prepared by reacting 1-olefins having the formula



10 where R is as hereinbefore described with formaldehyde and a halogenated compound selected from the hydrogen halides, thionyl halides, and carbonyl halides. These cyclic ethers can be prepared according to reaction conditions and procedures which are known to the art.

15 These lubricants can be applied to the surface of the metal by any conventional method known to one skilled in the art. Generally, the lubricant can be applied to the metal by Nalgene squeeze bottle. The amount of lubricant employed is only an amount sufficient to cover the surface of the metal to be worked.

20 The advantages of this invention are further illustrated by the following examples. The reactants, portions and other specific conditions are presented as being typical and should not be construed to limit the invention unduly.

#### EXAMPLE I

Threads on new stainless steel connectors using no lubricant, tightened up and backed out very easily with no pulling and galling.

30 Threads on used stainless steel connectors using no lubricant, tightened up and backed out with considerable pulling and galling.

35 Threads on used stainless steel connectors using a lubricant 4-chlorotetrahydropyran, tightened up and backed out with no pulling and galling. The used connectors were smoother threading after lubricating with 4-chlorotetrahydropyran.

The above example demonstrates the lubricating qualities of 4-chlorotetrahydropyran.

#### EXAMPLE II

40 Using an AE<sup>1</sup> coning tool, 1/4-inch OD<sup>2</sup> x 0.083 inch ID<sup>3</sup> 304<sup>4</sup> stainless steel tubing was cut using 4-chlorotetrahydropyran as a cutting lubricant. The cutting was every fast leaving a smooth surface on the tubing.

45 Threads were cut on the above-mentioned tubing using 4-chlorotetrahydropyran as a cutting lubricant. Threads were cut with little effort leaving smooth threads and collars, which tightened up and backed out with no dragging or binding.

50 This example again demonstrates the lubricating qualities of 4-chlorotetrahydropyran.

#### EXAMPLE III

55 Using 4-chlorotetrahydropyran as a lubricant for threading 3/4-inch 321<sup>5</sup> stainless steel, thread 3/4-inch 16 NF<sup>6</sup> dies ran very smoothly with no galling or dragging. Again, lubricating ability of 4-chlorotetrahydropyran is demonstrated.

1 Auto-Clave Engineers, Erie, Pa.

2 Outside diameter

3 Inside diameter

4 American Iron and Steel Type No.

5 American Iron and Steel Type No.

6 National Fine Thread

We claim:

1. A method of metal working comprising lubricating said metal working operations with a cyclic ether having the formula



wherein R is hydrogen or an alkyl or cycloalkyl radical or combinations thereof having up to and including 17 carbon atoms and X is a halogen.

2. The method of claim 1 wherein said metal working operations are threading, cutting and cutting threads.
3. The method according to claim 2 wherein said cyclic ether is 4-chlorotetrahydropyran.

**References Cited**

**UNITED STATES PATENTS**

|              |         |                |       |         |
|--------------|---------|----------------|-------|---------|
| 2,017,811    | 10/1935 | Cox            | ----- | 252—54X |
| 2,318,013    | 5/1943  | Prutton et al. | ----- | 252—54  |
| 10 3,275,555 | 9/1966  | Waight et al.  | ----- | 252—54X |

DANIEL E. WYMAN, Primary Examiner

W. H. CANNON, Assistant Examiner